

# UNITED STATES PATENT OFFICE.

WALTER DAGNALL, OF HAMPTON WICK, ENGLAND.

## PROCESS OF MANUFACTURING PARCHMENT-PAPER.

1,334,843.

Specification of Letters-Patent. Patented Mar. 23, 1920.

No Drawing.

Application filed February 4, 1919. Serial No. 275,006.

To all whom it may concern:

Be it known that I, WALTER DAGNALL, a subject of the King of Great Britain, residing at Hampton Wick, Middlesex, England, have invented certain new and useful Improvements in Processes of Manufacturing Parchment-Paper, of which the following is a specification.

The object of my invention is to treat paper so as to render it like parchment and waterproof, acid proof and of great strength.

For the purpose of my invention I use two baths of a mixture of sulfuric and sulfurous acid of different strength, viz. the first bath with sulfuric acid and water of a specific gravity of 1.700 to 1.800 to which is added sulfurous acid to reduce it until it registers 1.750 and the second bath, of which the sulfuric acid is of the same strength but the sulfurous acid is admixed in greater quantity to reduce it to a specific gravity varying from 1.200 to 1.400, all solutions being at about 60% F., the strength of the acid varying according to the quality and texture of the paper I wish to impregnate or parchmentize, *i. e.* the thicker the paper, the greater the strength of acid required. Then the paper is washed and afterward passed through an alkali bath and again washed and softened in any known manner either by glycerin, calcium chlorid, salt, or the like. In this latter process the paper or parchment may be loaded with any suitable material or mineral earth.

In carrying my invention into practice the paper is first run or passed from the reel into the first acid bath which is kept cool. It is then squeezed and the surplus acid returned to the first bath, it is then passed under rollers to the second bath (which is likewise kept cool,) squeezed between rollers, and the surplus acid returned to the second bath, care being taken that the specific gravity of the acid in these baths is in conformity with the limits above stated. It is essential that the acid baths do not rise above 60% F. since this would deteriorate the paper. The paper is then passed between water sprays and well washed to remove the acid, is then passed between rollers and squeezed, and then passed through an alkali bath to remove

any remaining acid that may be left in. 55 The paper is then passed between rollers and squeezed and again passed through water sprays and then between rollers and squeezed and then, if required, through the softening bath of glycerin, calcium chlorid, 60 salt, or the like (which latter bath may be heated by a steam coil). The paper is then squeezed again between rollers and finally dried, calendered and cut up ready for market. 65

By my invention the papers may be more thoroughly and quickly treated and at the same time thoroughly parchmentized, hence a greater quantity can be parchmentized within a given period than by known processes, which makes it more economical and hence cheaper to work and the parchment paper is of superior quality because of its not being brittle. 70

What I do claim as my invention, and 75 desire to secure by Letters Patent, is:—

1. Process of treating paper to render it like parchment, and waterproof, acid proof and of great strength, consisting in passing paper through a bath of sulfuric acid 80 and sulfurous acid and water, squeezing surplus acid from the paper, then passing the paper through a similar bath of less strength and squeezing out surplus acid, washing the paper in water, passing the 85 paper through an alkali bath to remove any remaining acid, squeezing the paper and again washing.

2. In a process of treating paper to make it like parchment, waterproof, acid proof 90 and of great strength, passing the paper through a bath of sulfuric acid and water of specific gravity of 1.800 admixed with sulfurous acid to reduce to a specific gravity of from 1.700 to 1.750, squeezing the 95 paper after leaving said bath, then passing the paper through a bath of sulfuric acid and water of specific gravity of 1.800 reduced by sulfurous acid to a specific gravity of from 1.200 to 1.400 at 60° F., 100 and then again squeezing the paper.

In testimony whereof I have hereunto set my hand in presence of two subscribing witnesses.

WALTER DAGNALL.

Witnesses:

J. M. BERTHELOT,  
Wm. A. BROWN.